

April 14, 1953

G. M. BEST

2,635,047

METHOD OF PROCESSING SOUND FILM

Filed July 27, 1949



Fig. 1.



Fig. 3.



Fig. 2.



Fig. 4.

GERALD M. BEST,  
Inventor

334 Val R. Goshaw

ATTORNEY

## UNITED STATES PATENT OFFICE

2,635,047

## METHOD OF PROCESSING SOUND FILM

Gerald M. Best, Beverly Hills, Calif., assignor to  
 Warner Bros. Pictures, Inc., Burbank, Calif., a  
 corporation of Delaware

Application July 27, 1949, Serial No. 106,993

1 Claim. (Cl. 95—5)

**1** This invention relates to the production of sound motion pictures, and particularly to methods of processing and printing sound records to accompany motion pictures.

In the production of composite motion picture film, the pictures and sound are first photographed and recorded, respectively, on separate films, which are separately processed and then eventually combined onto a single film for projection and reproduction. Two major types of sound recordings are in commercial use, one being the constant width, variable density type of record, and the other being a varying width, constant density type of record, also known as a "variable area" record. The present invention is directed to the variable area type of record, wherein distortion sometimes occurs in the form of a varying density component.

In the recording of film sound records, the film is sometimes subjected to undue strains and/or pressures which desensitize the original negative at the points of pressure or strain. For instance, should the film be curved sharply as it leaves the magazine, or any other point in its path between the supply reel and takeup reel, strains may occur therein, particularly between the sprocket holes or perforations. When such a negative is printed to a print, a varying density component is introduced, and, because of the occurrence of the sprocket holes, exhibits itself as a comparatively high level, 96-cycle tone, which renders the recording non-commercial. The variation in density may range from minus ten decibels to minus forty decibels. The present invention is directed to printing and processing methods for eliminating this variable density component, while providing a satisfactory commercial final print.

The principal object of the invention, therefore, is to facilitate the production of photographic film sound records.

Another object of the invention is to provide an improved method of eliminating a variable density component in a variable area type of photographic record.

A further object of the invention is to provide an improved method of printing and processing motion picture sound film to provide a satisfactory final print from an originally unsatisfactory negative record.

Although the novel features which are believed to be characteristic of this invention will be pointed out with particularity in the appended claim, the manner of its organization and the mode of its operation will be better understood

**2**

by referring to the following description, read in conjunction with the accompanying drawings, forming a part hereof, in which:

Fig. 1 is a graph showing H and D curves for different film emulsions on which the sound record is recorded and to which the sound record is printed, and

Figs. 2, 3, and 4 are partial sections of sound film illustrating the methods of the invention.

Referring now to the drawings, the original sound record negative used commercially for film sound recording is generally of the Eastman type 1372, with a base density of .31, and processed to a gamma of 3.70. Base density, as used herein, is the density of the Celluloid base on which the emulsion is coated at the factory. The H and D curve for this film is shown as curve A in Fig. 1. It has been found that, with the variation in density occurring from sharp bends in the film or other sources of pressure or strain, the density thereof ranges between a density of 1.5 to a density of 2.9, which variation is not detectable on the negative by the naked eye. This is illustrated in Fig. 2, wherein an unmodulated variable area film 1 with sprocket holes 8 is shown with bias lines 9, which have been exposed to light and in which no variation in density is discernible, but in which there can be a variation in density between 1.5 and 2.9. The width of the bias lines have been slightly exaggerated for better illustration of the invention.

This range of densities between 1.5 and 2.9 is shown by bracket 5 on curve A. Thus, the variable density component is not detected until the original sound negative is normally printed to an Eastman type 1302 film emulsion, which has a base density of .05. To provide the optimum sound record in normal processing, this print is developed to a gamma of 2.32, and the H and D curve therefor is shown at B. The density range of 1.5 to 2.9 now appears on the print between the range of the base density of .05 to .5, as shown by bracket 11. Since these densities represent a variation in output from the sound record range between approximately minus ten decibels to minus forty decibels, this 96-cycle variation has a level which renders the print non-commercial. This range of variation on the print is very easily discernible by the naked eye, as shown in Fig. 3, which is a print from the film of Fig. 2.

To eliminate this variable density component, chemical reduction methods have been used, but these are not commercially feasible for several

reasons, such as the expense involved because of the large amounts of reducing agents necessary, and the fact that these reducing agents are not always available, but must be prepared specially. Secondly, the variation in density is sometimes greater than can be satisfactorily handled by this method. On the other hand, the two methods to be described may always be applied by any laboratory in the normal course of commercial processing of film.

Referring again to the drawings and to further describe the invention, the print developed in accordance with curve B and shown in Fig. 3 is again printed to the same Eastman type 1302 emulsion to provide another print or what is known as a dupe negative, but which is developed to a gamma of 2.05, as shown by curve C. The first print shown by curve B is printed to a normal density of 1.85, while the dupe negative is printed to a normal density of 2.86. Normal density, as used in this description, is the density determined by cross modulation tests, as described by Baker and Robinson in the Journal of the S. M. P. E., volume 30, for January 1938. Non-technically, it is the density which produces the best possible sound prints as indicated by cross modulation tests. The normal density above stated provides a lighter than normal print, but which is the normal density best suited to eliminate the variable density noise component. The range of density variations causing distortion or noise has now been reduced to a narrow range between a density of 2.7 and 2.8, as shown by bracket 13. This dupe negative will appear similar to the original negative shown in Fig. 2, since the density variations occur above a density of 1.5.

The next step of the invention is to again make a print on emulsion 1302 from the dupe negative, as shown by curve E, at a normal density of 1.4. This final step will reduce the range of noise to such a small value as to be unmeasurable and unreproducible, since the limits will be practically the same as the base density of .05. The second print, therefore, will appear as shown in Fig. 4, the improvement therein being observable by comparing Fig. 4 with Fig. 3. Slight variations from these gammas and normal density values will provide satisfactory results. In the claim, three prints are mentioned, the duplicate negative being the second print, and the final or second print being the third print, while in Fig. 1, the second print referred to is the final print.

The above method has been found to be satisfactory in eliminating the variable density component as illustrated in Fig. 3; but, there has been some harshness in the sound when reproduced from the final print. To eliminate this harshness, a second process is provided which utilizes the "toe" of the characteristics, instead of the "shoulder," as just described.

Referring again to the drawings, we have the original negative processed in accordance with curve A and shown in Fig. 2, but this negative is now printed to Eastman type positive 1302 to a

lower gamma, such as 1.23, as illustrated by curve D. The normal density thereof is 1.0. This changes the variable density range of 1.5 to 2.9 to a range of .05 to .12 on the print, as shown by bracket 15 on curve D and illustrated in Fig. 3. From this print, a dupe negative is then made on the same emulsion developed to the same gamma, which transfers the density range from 1.14 to 1.20 on the dupe negative, shown by the bracket 16 on curve D. From this dupe negative, a second print is made with a normal density of 1.05, which reduces the density component of the second print to a variation which is so small as to be unreproducible and a noise level which is at the threshold of audibility in the neighborhood of minus forty decibels. This is illustrated in Fig. 4. Furthermore, not only is the noise eliminated, but the sound has substantially its normal quality as originally recorded.

These methods, therefore, provide satisfactory final commercial prints from non-satisfactory original negatives or prints, and which can be accomplished in the regular commercial laboratories with materials always available. The final commercial prints are used for rerecording to a composite master negative.

I claim:

The method of obtaining a variable area sound print having no variable density component from a variable area sound negative having such a variable density component, comprising printing said original negative to a first print for shifting said variable density component to the curved toe portion of the exposure density characteristic to reduce the range of said variation, printing a second negative from said first print to shift said range to an upper linear portion of the exposure density characteristic, and printing a second print from said second negative for shifting said variable density component to the curved toe portion of the exposure density characteristic to reduce the density range to an unmeasurable value, the emulsions of said first print, second negative, and second print being printed to a gamma of 1.23 at normal densities of substantially 1.0, 1.2 and 1.05, respectively.

GERALD M. BEST.

50 References Cited in the file of this patent

UNITED STATES PATENTS

| Number    | Name   | Date          |
|-----------|--------|---------------|
| 2,178,217 | Baker  | Oct. 31, 1939 |
| 2,352,032 | Steube | June 20, 1944 |
| 2,380,585 | Dippel | July 31, 1945 |

FOREIGN PATENTS

| Number  | Country       | Date         |
|---------|---------------|--------------|
| 473,115 | Great Britain | Oct. 6, 1937 |

60 OTHER REFERENCES

Roberts, "Photographic Duping of Variable-Area Sound," J. S. M. P. E., vol. 34, January 1940, pages 26-37.